

## UNITED STATES PATENT OFFICE

2,193,188

NONCAPILLARY SILK SUTURE AND METHOD  
OF PREPARING THE SAMETheodore F. Bradley, Stamford, Conn., assignor  
to American Cyanamid Company, New York,  
N. Y., a corporation of MaineNo Drawing. Application June 16, 1938,  
Serial No. 214,147

## 9 Claims. (Cl. 128—335.5)

The present invention relates to a method of making a noncapillary silk suture for surgical purposes and the suture per se.

Silk threads, made by twisting or braiding a number of degummed and cleaned raw silk filaments, have been used in surgery as suture material for many years. However, when such a silk suture is embedded in infected tissue, bacteria are harbored in its interstices and the suture becomes a nidus of infection which does not subside until the silk sloughs out or is removed surgically. Because of its capillarity, there is always the possibility of the exposed end of a silk suture acting as a wick to carry infection into the tissue.

15 The material, therefore, has never come into general surgical use for this purpose.

It is a principal object of the invention to produce a silk suture made of a number of silk threads, twisted, braided, woven or otherwise 20 associated together into a strand, which will be substantially noncapillary, and this object can most effectively be accomplished by coating such suture material with a composition which will present an unbroken surface to moisture.

25 The proposal to reduce the capillarity of silk sutures is not a new one. Many attempts have been made to this end and while it has been found not particularly difficult to treat a braided or twisted surgical silk so as to produce a satisfactory degree of noncapillarity, yet such treatment resulted in lending undesirable characteristics to the product or was unsatisfactory for other reasons.

30 A surgical silk suitable for use as a suture must be soft, pliable, nonacidic, noncorrosive and physiologically harmless and be capable of withstanding heat or chemical sterilization. These factors have generally stood in the way of the production of a successful noncapillary surgeons' silk, for any treatment which decreased capillarity was objectionable because such product did not meet the other necessary qualifications or because the stringent conditions of sterilization destroyed to at least some extent the surface coating which was responsible for noncapillarity.

45 The present invention, therefore, contemplates a noncapillary silk suture and a method of producing the same, whereby the product will not only be satisfactory from a completed stand-point, but will also stand up under sterilization treatment and maintain its desirable characteristics on storage and in the use for which it is intended.

To this end, the invention contemplates a 50 method of producing a substantially noncapillary

silk suture by applying to the silk suture stock, hereinafter referred to as a strand, a composition including ethyl cellulose in a volatile solvent and then permitting or inducing the solvent to evaporate. Under these conditions, the ethyl cellulose forms an unbroken film on the exterior periphery of the suture strand and even penetrates the same to a desired extent, whereby the capillarity of the strand is reduced.

A noncapillary suture thus produced will withstand the usual heat and/or chemical sterilization without substantial decrease in its noncapillarity. Where the sterilization treatment consists in contact with hot liquids, such as hot mineral oil, the suture will withstand the necessary high temperatures for the required periods without detrimental effect. Such heat sterilization treatment in oil is even beneficial in that it has a tendency to maintain the pliability of the suture, and in use even when the excess oil is 20 removed, a slight film thereof remains which, due to its water repellency, assists in maintaining the noncapillarity of the product.

The invention further contemplates a substantially noncapillary silk suture product in which 25 the silk strand or strands are provided with one or more coatings of ethyl cellulose with or without an additional superficial coating of oil.

A large number of coating and impregnating compositions were found to be satisfactory from the standpoint of actually reducing capillarity to the desired degree when applied to twisted or braided silk suture stock but resulted in lending stiffness, unpliability or other undesirable characteristics to the product, or the noncapillarity 30 was materially destroyed when such products were subjected to heat and/or chemical sterilization or to other conditions to which sutures may be normally subjected.

35 Ethyl cellulose was found to be of outstanding value in that it met all of the stringent requirements without producing detrimental effects while at the same time producing reduction in capillarity to the desired degree with optimum permanence.

In preparing the ethyl cellulose solution with which the silk stock is to be treated, ethyl cellulose of various viscosities and different solvents may be employed. While ethyl cellulose of viscosities of from 10 to 100 centipoises has been 40 found to be eminently satisfactory, yet a 20 centipoise grade has been found to be that most desirable.

45 Any volatile solvent for ethyl cellulose may be used for these compositions, such as the methyl

or ethyl ether of ethylene glycol, toluene, ethanol or mixtures thereof, as well as other known solvents, the proportions being varied to give the desired concentration of ethyl cellulose. Miscible diluents may also be employed and where these are noninflammable, such as carbon tetrachloride, their use may be desirable under some circumstances.

The preferred coating composition comprises 10 the following substances in substantially the proportions specified:

*Solution A*

|                                        | Grams            |
|----------------------------------------|------------------|
| 15 Ethyl cellulose—20 centipoise grade | 40               |
| Toluene                                | 120              |
| Ethanol                                | 40               |
| 20                                     | 200 (20% solids) |

*Solution B*

|               | Grams           |
|---------------|-----------------|
| 25 Solution A | 40              |
| Ethanol       | 10              |
| Toluene       | 50              |
| 30            | 100 (8% solids) |

30 Suture stock silk may then be immersed in, sprayed or otherwise contacted with, such a solution for from one to two minutes, the excess solution removed and then the coated strand air-dried or preferably at some elevated temperature 35 to remove all of the volatile solvent. This operation may be repeated as many times as necessary in order to produce a coating of the desired thickness or weight, dependent upon the circumstances. In order to reduce fire hazard 40 due to the inflammability of the above solvents, requisite amounts of carbon tetrachloride may be added thereto as desired.

After the silk has thus been treated to render it 45 noncapillary, it may be cut into the required lengths, wound into small coils, placed in glass tubes, which are filled with a light mineral oil and then sealed by fusion of the glass, the sealed tubes may then be placed in an autoclave and heat sterilized. When this is complete, the tubes 50 are ready for packaging. While the above method of sterilization is preferred, other standardized procedures may likewise be employed.

55 While the invention has been described with specific reference to certain embodiments, it is to be understood that it is not to be limited thereto but is to be construed broadly and restricted solely by the scope of the claims.

I claim:

1. A substantially noncapillary non-water absorptive silk suture comprising a silk strand coated with a composition including ethyl cellulose, and capable of maintaining its noncapillarity at no substantial loss after having been heat sterilized in mineral oil. 5

2. A substantially noncapillary non-water absorptive silk suture comprising a silk strand coated with ethyl cellulose and having a superficial exterior coating of oil. 10

3. A substantially noncapillary non-water absorptive silk suture comprising a silk strand coated with ethyl cellulose and having a superficial exterior coating of mineral oil. 15

4. A method of making a substantially noncapillary silk suture which includes the following steps: contacting a silk strand with a solution of ethyl cellulose in an organic solvent, removing the strand from the solution and evaporating the solvent from the ethyl cellulose so as to produce an adherent coating of the latter on the strand. 20

5. A method of making a substantially noncapillary silk suture which includes the following steps: immersing a silk strand in a solution of ethyl cellulose in an organic solvent, removing the strand from the solution, removing the excess solution from the strand and drying the strand. 25

6. A method of making a substantially noncapillary silk suture which includes the following steps: immersing the silk strand in ethyl cellulose dissolved in a mixture of toluene and ethyl alcohol, removing the strand from the solution and drying the strand. 30

7. A method of making a substantially noncapillary silk suture which includes the following steps: immersing the silk strand in a solution of 20 centipoise viscosity ethyl cellulose in an organic solvent, removing the strand from the solution and drying the strand. 40

8. A method of making a substantially noncapillary silk suture which includes the following steps: immersing a silk strand in an 8% solution of 45 20 centipoise viscosity ethyl cellulose in an organic solvent, removing the strand from the solution and drying the strand.

9. A method of making a substantially noncapillary silk suture which includes the following steps: immersing a silk strand in a solution of ethyl cellulose in an organic solvent, removing the strand from the solution and evaporating the solvent from the ethyl cellulose so as to produce an adherent coating of the latter on the strand 50 and sterilizing the coated strand in mineral oil. 55

THEODORE F. BRADLEY.